

R. A. HADFIELD AND A. G. M. JACK,  
CAP FOR ARMOR PIERCING PROJECTILES.  
APPLICATION FILED MAY 26, 1914.

1,310,073.

Patented July 15, 1919.

Fig. 1.



Fig. 2.



Fig. 3.



Witnesses:

J. M. Millward  
M. L. Breslin

Robert A. Hadfield, Inventor  
Alexander G. M. Jack,  
By their Attorney  
Alfred Wilkinson

# UNITED STATES PATENT OFFICE.

ROBERT ABBOTT HADFIELD, OF WESTMINSTER, LONDON, AND ALEXANDER GEORGE MACKENZIE JACK, OF SHEFFIELD, ENGLAND.

## BEST AVAILABLE COPY CAP FOR ARMOR-PIERCING PROJECTILES.

1,310,073.

Specification of Letters Patent. Patented July 15, 1919.

Application filed May 26, 1914. Serial No. 840,984.

To all whom it may concern:

Be it known that we, Sir ROBERT ABBOTT HADFIELD, knight, F. R. S., and ALEXANDER GEORGE MACKENZIE JACK, subjects of the 5 King of Great Britain and Ireland, residing, respectively, at Westminster, in the county of London, England, and Sheffield, Yorkshire, England, have invented Improvements in or Relating to Caps for Armor-Piercing 10 Projectiles, of which the following is a specification.

This invention relates to caps for armor piercing projectiles and consists in the discovery that a great improvement in the penetration of armor plate may be effected by hardening the cap to a limited degree in distinction to the very high degree heretofore described and practised and that the improved result may be accomplished by a 20 cap of comparatively small size.

The function of the cap is primarily to support the point of the shot itself so that it will not be broken down at the instant of impact, and also, if possible, to effect initial 25 penetration, or weakening, of the plate, and thereby prepare the way for the shot itself and make penetration easier.

Heretofore the hardening of caps has been suggested and such caps have been practically used to some extent but a very high degree of hardening was aimed at, approaching or equaling the hardness of the armor-plate itself. So far as we know it has never occurred to anyone that this high degree of 35 hardness was not the most desirable, much less that a better effect could be obtained by lowering the hardness. This high degree (sometimes described as "glass scratching" hardness) was about or above 610 on the 40 Brinell ball scale, possibly much higher.

After years of study and experiment and many tests, we however, have found that the aforesaid high degree of hardness applied to caps tends to produce brittleness, so that 45 there is great danger of the caps shattering at impact, even if the cap be large, without affecting the plate, or even fulfilling the purpose of sustaining the point of the projectile, so that the projectile may pass unbroken 50 through the plate. But on the other hand we have discovered the fact, which at first thought would seem extraordinary, that a substantially lower degree of hardness is much more effective and that a cap har-

dened to a degree substantially below that 55 high degree above referred to will not only reinforce the point of the shot itself but will initially perforate the plate or at least start the fracture thereof.

A degree of hardness not above about 560 60 is substantially below said glass-scratching or dead hardness and gives greatly improved results, but we recommend a hardness of about 515 to about 525. This degree of hardness should be aimed at as being about the 65 best but the improved results may be obtained by an approximation thereof, even as low as about 460 to 470 and therefore we specify the last named degree as about the 70 lowest that will bring the cap within the limits of our invention.

This limited hardening prescribed by us is so substantially below the high degree heretofore aimed at and gives such characteristically new and improved results, that 75 we prefer to refer to our caps and to their peculiar degree of hardness as "stiffened" and "stiffness" to distinguish from "hardened" and "hardness" for this seems to us a better descriptive term and better to indicate the difference from the old caps. 80

We have also discovered that it is better to reduce the extent of the "stiffness" or the amount of the "stiffened" material; we prefer that it should not amount to over about 85 five (5) to about ten (10) per cent. of the whole cap; in some cases not over about three (3) to four (4) per cent., whereby we have been able greatly to reduce the size of the caps and to attain successful results with 90 small caps. And diminution in the size of the cap is important, for, to preserve the ballistics, the total weight of the projectiles must not vary, and the weight of the cap is just so much taken from the weight of the 95 shot itself, and by so much is reduced the capacity of the shot to perforate, as well as the size of the powder chamber, the strength of the wall, etc. Therefore even a slight diminution in the size of the cap becomes 100 important for the weight subtracted from the cap may be added to the weight of the shot itself.

In other words the important feature of our invention is the discovery that a cap 105 having a stiffened tip will set back the plate or start the perforation thereof better than an ordinary unhardened cap, but that the

degree of hardness must be limited, for if carried too far, that is to or approaching a hardness of about 610, the purpose of the 5 hardening is largely defeated, for the cap is lacking in the requisite quality of resistance to splitting or shattering, wherefore it breaks at the instant of impact with little effect on the plate and is inferior to the ordinary cap. But if, on the other hand, the 10 cap is hardened or "stiffened" to a degree substantially below 610 it will not shatter at impact, but will be hard enough to start the perforation of the plate and thereby cause the same shot much more effectively to perforate 15 the plate, whether fired normally or obliquely, than has ever before been accomplished. Furthermore, the cap so hardened may be greatly reduced in size without reducing its effectiveness and a more or less 20 gradual diminution from the "stiffened" front portion rearwardly toward the point of the shot is advised.

The better to explain our invention, reference is made to the drawings herewith. 25 Figure 1 thereof shows in longitudinal section a cap of desirable shape and a portion of the shot to which the cap is applied. Fig. 2 is a similar section, much reduced in scale, showing the entire shot to illustrate the 30 small size of the cap. The shape of the cap here shown is desirable but we do not limit ourselves to that shape for our invention can be applied with excellent results to caps of various shapes, conical, pointed, 35 rounded or of other desired shape. Fig. 3 is a view similar to Fig. 1 showing a modification.

In Fig. 1 we have indicated the degree and extent of the hardening and the gradual diminution thereof rearwardly toward the point of the shot. While it is of course not possible to harden the cap with absolute accuracy as to degree and extent, yet the results here indicated are approximately 40 correct. A indicates the hardened or stiffened front portion of the cap; this is the cross hatched portion varying somewhat in extent. Good results have been attained with this stiffened portion not over about 45  $3\frac{1}{2}\%$  of the entire cap. The hardness of 50 this portion will vary somewhat and it can not be of absolutely uniform hardness but as aforesaid we should place the limit at not above about 560. Projectiles have attained 55 excellent results, as hereinafter described, with this portion stiffened from about 475 to 515.

In zone B, whose extent is roughly indicated by the lines C to D, the hardness will 60 be less, that is desirably from about 490 to about 450. In zone E, approximately outlined by the lines D and F, the hardness will gradually diminish from 450, the bulk of this zone being from about 400 to about 65 350. The hardness of the bulk of the re-

mainder behind about the line F will be much lower, varying from 250 to 220 down to about 190 more or less.

While the essential feature of the invention is the "stiffening" of the front portion 70 of the cap as aforesaid, we recommend in addition a gradually diminishing hardness from said front "stiffened" portion rearwardly toward the point of the shot, substantially as described, so that the portion 75 of the cap adjacent said point shall be soft and tough, or comparatively soft. From this it results that upon impact of the capped projectile with the plate the hard point of the shot will pass through cap material of gradually increasing stiffness, or 80 hardness, and will reach and perforate the plate without being suddenly subjected to contact with the extremely hard surface of the armor plate. As a result the point of 85 the projectile is supported, until it enters the plate, with a gradually increasing pressure from the moment of impact of the cap tip with the hard surface of the plate, and the sudden shock to which the point of the 90 projectile is usually subjected in passing through the relatively soft metal of the cap and striking the hard metal of the plate, is avoided, greatly reducing the danger of fracturing the point of the shot. 95

The cap may be stiffened by any suitable method, for instance by heating up to a temperature of about  $850^{\circ}$  C. and then quenching in water or other suitable medium for a sufficient time. Or even may be over-hardened and then tempered to reduce the 100 hardness to the desired degree, though we do not recommend this latter method.

We do not propose to limit ourselves to any particular composition of metal for the 105 cap, for any well known material may be used, for instance a steel containing a sufficient amount of carbon, nickel and chromium to permit the end or tip of the cap to be stiffened leaving the bulk of the remainder of the cap tough and relatively soft. We do not mean by this to imply that the toughness of the front portion is reduced for on the contrary one of the great 110 advantages attained by our invention is that 115 said front portion is maintained at a high degree of toughness. Excellent results have been attained in tests with projectiles provided with our new cap. In certain recent 120 tests several 14" projectiles fitted with our new cap having a weight of  $7\frac{1}{2}\%$  of the total projectile weight, perforated unbroken a K. C.  $13\frac{1}{2}$  inch plate inclined at ten degrees. Other tests have since been made with shot 125 of comparatively an old type; these tests were made obliquely. Some of the shot were fitted with the ordinary cap; some with the cap described in this application in weight only  $3\frac{1}{2}\%$  to 4% of the total weight of the projectile. The shot fitted with the new cap 130

went through unbroken; those with the old cap broke up badly, leaving one third in front of the plate.

So far as we are informed the highly hardened caps heretofore in use have been made very large in the endeavor to prevent the shattering above described, and even those have not been very successful, much less so than our stiffened caps, which are also of small size.

In the process of stiffening our caps, it is possible that in some cases a trifling thickness of the metal at the point might be found to be hardened above the degree specified by us, but such would be a superficial hardening of only the skin portion of the cap and would not be a substantial modification of the stiffened condition prescribed by us, nor a departure from our invention.

What we claim is:

1. A cap for an armor piercing projectile having its front portion stiffened to from about 460 to about 560 ball hardness and gradually diminishing in stiffness rearwardly from said front portion.

2. For an armor piercing projectile, a cap having a stiffened tip the weight of which is of the order of from three to ten per cent. of the weight of the whole cap and the hardness of which corresponds substantially to a ball hardness of from about 460 to 560.

3. An armor piercing projectile comprising a projectile proper and a cap having a stiffened and toughened tip or forward end, the final stiffness corresponding to a ball hardness of the order of from about 460 to 560 and the weight of such stiffened portion being of the order of from about three to ten per cent. of the weight of the cap.

4. For an armor piercing projectile, a cap having a stiffened tip, the stiffness thereof corresponding to a ball hardness of not over about 560 and substantially below glass scratching hardness, and the portion of the cap adjacent the tip being of gradually diminishing hardness, the narrow zone at the front end being from about 560 to 475 ball hardness, the next zone being of about 490 to about 450, the bulk of the next zone being from about 400 to about 350, and the remainder of the cap being from about 250 to 190, said zones being approximately of equal width, and the three zones occupying not more than one-half the bulk of the cap from the extreme tip to the portion to lie in contact with the tip of the projectile.

5. For an armor piercing projectile a cap having its tip hardened or stiffened to a high degree, but not above about 560 ball hardness.

6. For an armor piercing projectile, a cap having its tip stiffened to about 515 to 525 ball hardness.

7. For an armor piercing projectile, a cap having its tip stiffened to a high degree, but not above about 560 ball hardness, and gradually diminishing in stiffness rearwardly from said tip.

8. For an armor piercing projectile, a cap having its tip very tough and stiffened to from about 460 to 560 ball hardness, the remainder of the cap being very tough but comparatively soft.

9. For an armor piercing projectile, a cap having its tip stiffened to from about 460 to about 560 ball hardness and being in weight from about  $3\frac{1}{2}\%$  to about  $7\frac{1}{2}\%$  of the entire projectile.

10. A cap for an armor piercing projectile, the portion of which that will be forward of the point of the projectile to which the cap is to be fitted, is of gradually increasing stiffness in a forward direction, the final degree of stiffness adjacent to the point or tip of the cap corresponding to a ball hardness of the order of about 560.

11. A cap for an armor piercing projectile, the portion of which that will be forward of the point of the projectile to which the cap is to be fitted, is of gradually increasing stiffness in a forward direction, the final degree of stiffness adjacent to the point or tip of the cap corresponding to a ball hardness of the order of about 560, the stiffened portion of the cap, corresponding to a ball hardness of 450 to 560, not constituting more than about three and one half per cent. of the entire cap.

12. A cap for an armor piercing projectile, having its front portion stiffened to from 450 to 560 ball hardness and gradually diminishing in stiffness rearwardly from said front portion, said stiffened cap weighing about three and one half per cent. to about seven and one half per cent. of the weight of the projectile.

13. A cap for armor piercing projectile, made of nickel chromium steel and having its front portion stiffened to from about 460 to 560 ball hardness and gradually diminishing in stiffness rearwardly from said front portion.

Signed at 22 Carlton House Terrace, Westminster, England, this thirteenth day of May, 1914.

ROBERT ABBOTT HADFIELD.

ALEXANDER GEORGE MACKENZIE JACK.

Witnesses:

LEONARD ROWLAND,  
E. S. HEAP.